

## UNITED STATES PATENT OFFICE

2,029,968

## MANUFACTURE OF TEXTILES

Leo Wallerstein, Rowland A. Gale, and Thomas G. Hawley, Jr., New York, N. Y., assignors to Wallerstein Company Inc., a corporation of New York

No Drawing. Application April 26, 1934,  
Serial No. 722,504

## 6 Claims. (Cl. 117—2)

The present invention relates to a method of manufacturing textiles and it particularly relates to a method of manufacturing textiles containing natural silk in gum.

5 In the production of many textile materials, and particularly in the case of textile materials containing or composed of natural silk in gum, it has been found desirable to have the textile fibres possess greater body during the knitting and/or 10 weaving operation than is possessed by the final fibres or threads in the finished fabric. This is attained in the case of natural or raw silk by utilizing the silk in the condition which it is produced in nature with the filaments or strands 15 of the silk containing the gum or bast naturally placed thereupon.

Although this gum, bast or body-giving coating, naturally occurring upon the fibres or artificially placed thereupon, is desirable during the 20 textile forming operations, before the textile is finished, it should be removed without disadvantageously affecting the strength, surface, appearance, or other characteristic properties of the fabric.

25 In the case of fabrics containing natural silk with gum, it has been customary to degum the woven or knitted fabric by placing it in a boiling soap solution which will have the effect of removing gum, thereby preparing the fabric for such 30 other finishing operations as may be required, as for example, dyeing, bleaching, and/or printing.

In many fabrics, however, certain threads or 35 yarn making up the fabric have been previously processed before weaving or knitting and/or during the weaving or knitting process so that the gum thereon becomes relatively inaccessible to the dissolving action of the degumming bath.

40 In satin fabrics, for instance, all or part of the warp threads are woven in such a manner as to extend over a great many filling threads and lie for substantial distances upon the face of the fabric in a position where they are relatively more exposed to the action of the degumming 45 bath than the residual closely intermeshed and interwoven warp and/or weft threads.

When satin fabrics of this character are subjected to the action of a degumming bath, the 50 gum from the exposed overlying portions of the warp threads will be more readily removed, while the gum from the intermeshed and interwoven residual warp and weft threads will be relatively slowly removed. As a result, these overlying threads are necessarily subjected to an excessive 55 amount of treatment in the degumming bath in

order that the fabric as a whole shall be completely degummed.

In the case of certain crepe weaves also the weft or filler threads are relatively highly twisted, while the warp threads have a relatively low 5 amount of twist. When a crepe fabric of this character is subjected to the degumming bath, the warp threads where exposed are readily degummed, whereas the higher twisted weft or filling threads and portions of the warp threads 10 are only relatively slowly degummed, as a result of this difference in accessibility to the degumming solution. The warp threads in this case also will be over-treated and consequently damaged or rendered liable to damage in the degumming 15 solution before the twisted weft or filling threads are completely degummed.

Again in the case of yarns for forming knitted fabrics, particularly in forming stockings, certain of the strands making up the final knitting yarn 20 have sometimes been given a relatively high twist, while other strands are given a relatively low twist or substantially no twist at all. In this instance, again, the untwisted or low twist strands will be degummed at a much faster rate than the 25 relatively highly twisted strands.

It is the plan of the present invention to so prepare textile fabrics containing natural silk in gum, that the various filaments, threads or fibres 30 of silk in gum making up the same will be degummed in more nearly the same time periods, thus eliminating the need of over-treating one portion of the fabric because of the difficulty of degumming another portion.

The object is to prepare an improved textile 35 fabric, having a relatively untwisted or low twist warp and a relatively high twist filling or weft which may be degummed in a relatively shorter time without necessitating a long boiling period due to the relative inaccessibility of 40 the gum on the highly twisted weft or filling threads.

Another object is to prepare a satin fabric, preferably containing in whole or part natural silk in gum which may be subjected to degumming treatment 45 without the overlying warp threads being disadvantageously affected due to their accessibility by reason of any extended treatment necessary because of the relative inaccessibility of the filling or weft threads.

Another object is to provide twisted yarns for knitting and for other purposes in which, although the various fibres making up the yarn have different amounts of twist, it will not be necessary to over-treat these threads of relatively 50 55

low twist, the gum of which is relatively accessible to the degumming action in order to secure satisfactory degumming of the threads of relatively high twist, the gum of which is not readily accessible.

Other objects will appear during the course of the following application.

According to the preferred embodiment of the present invention, it has been found desirable to 10 prepare the yarn or fibres which are to be so processed or placed in the fabric that their gum or bast is relatively inaccessible to the degumming bath, that they may be degummed at more nearly the same rate as the yarn or fibres, which 15 are so processed and/or placed in the fabric that their gum coating will be relatively accessible.

As a result when some fibres are twisted and/or so interwoven in the fabric that their gum coating will be less accessible than the gum coating 20 of the other strands, fibres or yarn, the degumming action will take place at a more uniform rate, with the result that both the inaccessible and accessible fibres, strands, or yarn, will be degummed in the fabric at more nearly the 25 same rate without the need for over-treating the accessible fibres with its accompanying disadvantageous effects.

According to the present invention, it has been found most suitable and desirable to resort to an 30 impregnation of the yarn before twisting, knitting and/or weaving with a proteolytic enzyme preparation under such conditions, as not to degum the yarn.

Among the preferred enzyme preparations are 35 those prepared from plants and/or by the growth of certain bacteria, fungi, and other similar organisms.

It has been found most suitable, especially in use of plant enzymes, such as papain, to use activators, such as sulphur compounds or cyanides.

With enzymes of bacterial origin, it has been found suitable to add sodium and potassium carbonates or bicarbonates, or mixtures thereof.

It is an essential feature of the present invention that the natural silk in gum before being subjected to any textile operations, such as twisting, knitting, and/or weaving, be impregnated with the enzyme without being substantially degummed. The degumming operation is only 45 carried out after the enzyme impregnation and may be carried out without the utilization of any additional proteolytic enzyme preparations and after the goods have been finally woven and knitted and are being subjected to or about to 50 be subjected to finishing operations.

In the preferred procedure, the natural silk in yarn or skein form, is dipped into a bath of a temperature below 50° C., said bath containing in 55 solution and/or in suspension the proteolytic enzyme preparation with which may be preferably combined the alkali metal salt or salts of a high molecular weight fatty acid or fatty acids, or the alkali metal salts of sulphuric or sulphonic acids of aliphatic, aromatic, and/or alicyclic compounds of high molecular weight and/or sulphonated oils and raw oils.

Among the wetting out compounds which may be used are soaps such as sodium oleate, sodium palmitate, sodium stearate, sodium hexadecyl sulfonate, and so forth; and sulphonated oils such as sulphonated olive oil, sulphonated castor oil and sulphonated cocoanut oil.

To this bath is preferably also added a raw oil 75 as for example neat's-foot oil, olive oil, or other

similar vegetable, mineral or animal oils and so forth.

The skein or yarn may be suspended in the soaking bath for a sufficient length of time to assure that the enzyme preparation and the other ingredients have thoroughly penetrated the gum in the silk, and at all times the temperature and pH should be so maintained that substantially no degumming action results.

This soaking may be carried out from 30 minutes to 16 hours and it preferably should not be carried out for longer than 24 hours. The skein or yarn after being so impregnated with the enzyme preparation is centrifuged so as to remove excess moisture and then is partly or thoroughly 15 dried before being subjected to further textile forming operations.

Various protease preparations may be used in carrying out the process, such as protease preparations derived from micro-organisms which 20 under suitable culture conditions develop proteolytic enzymes, as, for instance, preparations derived from aspergillus oryzae, and/or from cultivation of bacteria, such as belong to the group of mesentericus or subtilis. Other suitable 25 proteolytic enzymes may be used, such as papain, trypsin, pancreatin, or pepsin. Suitable mixtures of the described enzymes may be used.

As examples in carrying out our process, we may proceed as follows:

*Example 1.*—100 pounds of raw silk are soaked from 30 minutes to 1 hour in a bath or solution consisting of 400 pounds of water in which have been dissolved 50 pounds of the bacterial enzyme preparation, 1 pound of sodium sulfite or sodium 35 bicarbonate for effecting a suitable pH, and 1 pound of sulfonated oil, this latter material being used to effect a better penetration, or as it is technically called, a wetting-out of the fiber, though it will be understood that other penetrants can be 40 used for effecting this wetting-out, such as a small amount of soap. Other suitable pH regulators, for instance, sodium carbonate, or a mixture of both may be used instead of the sodium sulfite referred to.

Soaps and emulsions of common soaking oils, such as neat's-foot oil may also be used in conjunction with enzymes. The temperature at which this process is carried out may be advantageously varied with the time consumed in the 50 operation, the nature or origin of the silk, the nature of the particular enzyme employed, and the presence of other constituents, such as pH regulators. However, we generally employ this process at room temperature, that is, from 60° to 45 90° F.

The silk is then removed from the enzyme bath and the adhering liquor is removed in any suitable manner, as by centrifuging, and after the centrifuging step the silk fibers are dried at a low 60 temperature by an air blast or any other suitable method.

*Example 2.*—100 pounds of 13/15 Japan white silk in the gum are soaked for 30 minutes at room 65 temperature in 400 pounds of a water solution containing 5 pounds of papain, 4 pounds of sulfonated oil, 0.05 pounds of potassium cyanide, 2 pounds of mono-sodium phosphate. It is then centrifuged and air dried.

*Example 3.*—100 pounds of 13/15 Japan white silk in the gum are soaked for 30 minutes at room 70 temperature in 400 pounds of a water solution containing 5 pounds of pancreatin, and 1 pound of sodium sulfite or sodium bicarbonate and suit- 75

able penetrants and/or oils. It is then centrifuged and air dried.

If desired, in the above examples, the time of soaking or impregnation may be increased to 8 to 16 hours or overnight and the amount of the enzyme preparation may be cut in half. The pH of the impregnating baths is preferably regulated at all times to be between 4 and 10 and temperature to between 60° and 90°.

10 After the silk has been impregnated in this manner without any substantially visible effect upon the gum, the silk may be processed by winding and twisting, and it may be subsequently woven either alone or with other materials.

15 For example, the silk skeins so impregnated may be processed into a highly twisted silk yarn containing between 20 to 80 turns. This yarn is to be utilized for the filling of crepe fabric having a relatively untwisted warp which has not 20 been so impregnated. With such a crepe fabric when subjected to a treatment in a hot or warm degumming bath, it has been found that not only may the crepe fabric be degummed at a substantially rapid rate and in a much shorter time than 25 a similar fabric in which the twisted filling has not been previously impregnated, but in addition the resultant fabric is of improved quality being whiter and having no appreciable chafing or damage.

30 With a satin fabric on the other hand the filler may be conveniently previously impregnated, as above described, while the relatively accessible and exposed overlying strands are not impregnated. Where part of the backing has been relatively highly twisted, while another portion of the backing is either untwisted or only of low twist character, the former may have been subjected to an impregnation at a greater concentration or for a greater length of time with the same 35 preparation as above described, while the latter may be subjected to a lesser enzyme concentration or to treatment in the soaking bath for a lesser period of time. As a result of this treatment the various strands of the satin fabric will degum at more nearly the same rate, permitting the entire degumming operation to take place in a shorter time and produce a much higher quality fabric.

As a general rule, when fabrics contain relatively accessible and inaccessible strands and filaments, the inaccessible strands of which have been impregnated with an enzyme preparation, as above described, they may be degummed, in many instances in about half the time to quarter 50 the time of fabrics in which neither the inaccessible nor the accessible portions thereof have been subjected to such impregnation.

As above indicated, where different portions in the fabric have relatively different degrees of accessibility in respect to the decoating or degumming bath, the fibres making up the different portions may be differentially impregnated with the enzyme preparation either in respect to time or concentration so that in the final decoating or degumming bath the process will take place in a more rapid fashion without over-treatment of any particular portion of the fabric.

To give several examples of the degumming of fabrics which have been differentially impregnated according to the present invention:

Example 1.—A crepe back satin is formed of a warp consisting of 20—22 yellow japan silk in single threads not twisted together and not treated with proteolytic enzymes, which are woven so 75 as to lie predominantly on the surface of the fab-

ric; and of a filling or weft consisting of threads of 13—15 white japan silk which have been treated with proteolytic enzymes and which also have been twisted together. In the filling, the single threads, after having been treated with an enzyme preparation and dried are twisted together, eleven at a time, to a twist of fifty turns per inch.

These composite strands are woven with the warp using alternately two right and two left twist strands.

The woven fabric is degummed by immersion in a solution containing 150 lbs. of soap and 150 lbs. of sodium sulfite in 2,000 gallons of water at a temperature of 208—212° F.

Satisfactory degumming without chafing of 15 the fabric results in one hour.

In the case of a fabric of identical construction, but in which the filling thread were not especially prepared with enzymes, as outlined above, two hours' treatment in the degumming 20 solution was required and the resulting fabric showed definite defects due to chafing of the exposed warp threads.

Example 2.—A flat crepe is formed of a warp consisting of 20—22 yellow japan silk single 25 threads, 324 per inch, not twisted, and not treated with proteolytic enzymes; and of a filling or weft consisting of 2 right and 2 left hand twisted threads woven alternately at 56 threads per inch. The threads were made by twisting together three 30 threads of 13—15 white japan silk which had been impregnated with a proteolytic enzyme preparation. They were twisted 60—65 turns per inch.

The fabric was degummed in a boiling 2% soap 35 solution in 15 minutes. It was white in appearance and soft. The corresponding fabric made without the proteolytic enzyme treated silk required over 40 minutes boiling in 2% soap solution for complete degumming. Its appearance 40 was of a yellowish cast.

By the expression inaccessible fibres as contrasted with accessible fibres, or by similar expressions applied to filaments, strands, yarn, and so forth, is meant those fibres having a body-giving coating, whether of a protein, carbohydrate, and/or fatty character, which have been processed or positioned in such a manner in the final fabric that they are relatively inaccessible to the action of degumming or decoating solutions.

This inaccessible positioning or locationing of the coating is usually caused by the processing of the fibres, strands, filaments, and/or threads carrying the coating, particularly by twisting or 55 by interlacing, interweaving, and/or interknitting such filaments, strands, and fibres that their coatings are relatively inaccessible as contrasted to the coating of other fibres in the fabric.

The present application is a continuation in 60 part of application Serial No. 606,286, filed April 19, 1932 and is similar in subject matter to co-pending applications Serial No. 722,505 to 722,-508 all inclusive, filed April 26, 1934, all of which applications are being issued concurrently on 65 February 4, 1936.

The present application is particularly directed to fabrics including natural silk in gum in which some of the gum is in relatively inaccessible condition, and in which this gum has been impregnated with a proteolytic enzyme as described.

What is claimed is:—

1. A process of making a fabric containing natural silk fibres provided with their body-giving gum coatings, some of which coatings in the 75

- fabric are in relatively inaccessible condition, while others are in accessible condition to the action of a subsequent decoating bath, which comprises impregnating these fibres, the coatings of which are relatively inaccessible with a proteolytic enzyme preparation without removing said coating, drying said impregnated fibres, combining said impregnated fibres with unimpregnated fibres, the coatings of which are relatively accessible to form a fabric.
2. A process of forming crepe silk fabrics of natural silk in gum, which comprises impregnating the filling yarn with a proteolytic enzyme preparation without removing said gum, dehydrating said impregnated yarn, highly twisting this filling yarn and then weaving this highly twisted yarn with a relatively untwisted unimpregnated warp yarn.
3. A process of preparing satin fabrics of natural silk in gum, which comprises impregnating the filling yarn with a proteolytic enzyme preparation without removing said gum, dehydrating said impregnated yarn, and weaving such impregnated yarn together with unimpregnated textile fibres making up the overlying warp.
4. A process of preparing satin fabric of natural silk in gum with a twisted filling yarn and an untwisted overlying warp yarn which comprises impregnating the filling yarn before twisting with a proteolytic enzyme preparation without removing said gum, dehydrating said im-

pregnated yarn and weaving such impregnated yarn together with unimpregnated textile fibres making up the overlying warp.

5. A process of making fabrics of composite twisted yarns, of natural silk in gum, in which some of the strands are relatively highly twisted while other of the strands are relatively lowly twisted or untwisted, which comprises previously impregnating those strands, which have been relatively highly twisted with a proteolytic enzyme preparation without degumming, drying the impregnated strands, and then combining said impregnated strands with the unimpregnated strands of relatively low twist or untwisted to form a textile fabric therefrom.
6. A textile fabric composed of a plurality of interconnected fibres composed of natural silk in the gum, some of which fibres have been so mechanically processed as to render the coatings relatively inaccessible to a degumming bath and other of which fibres have been so processed as to render their coatings relatively accessible to a degumming bath, said inaccessible fibres having been previously impregnated with and containing a proteolytic enzyme preparation without removing said gum and said accessible fibres being unimpregnated.

LEO WALLERSTEIN.

ROWLAND A. GALE.

THOMAS G. HAWLEY, JR. 30